

## UNITED STATES PATENT OFFICE

GEORGE HOLLAND ELLIS AND HENRY CHARLES OLPIN, OF SPONDON, NEAR DERBY, ENGLAND, ASSIGNEES TO CELANESE CORPORATION OF AMERICA, A CORPORATION OF DELAWARE

## MANUFACTURE OR TREATMENT OF TEXTILE OR OTHER MATERIAL

No Drawing. Application filed January 6, 1931, Serial No. 507,046, and in Great Britain March 5, 1930.

This invention is a continuation in part of United States application S. No. 415833 of 21st December, 1929 and relates to the treatment and also to the manufacture of artificial silk and other filaments or products and to the treatment of yarns, fabrics or other materials made of or containing filaments or other products produced from solutions of cellulose esters or ethers.

10 The said prior United States application describes processes for the treatment of materials made of or containing filaments or other products produced from solutions of cellulose esters or ethers with steam, where-  
 15 by already delustered materials or materials of low lustre are rendered lustrous, and by continuing the treatment sufficiently the materials may be rendered non-delusterable on treatment with hot aqueous liquids or moist steam. The said prior United States application indicates that it is preferable to em-  
 20 ploy temperatures of steam approximating to or slightly above the boiling point of wa-  
 25 ter at the pressure used, though it is stated that higher temperatures may be employed.

The present invention relates more partic-  
 30 ularly to rendering delustered materials or materials of relatively low lustre, such as are treated according to the processes of the said prior United States application, with steam so as to increase their lustre. We have now found that in this particular application of the processes of the said prior United States application considerable advantages accrue  
 35 from effecting the treatment with superheat-  
 ed steam. The steam may be employed at atmospheric pressure but preferably it is used at a higher pressure, and in any case is superheated. The temperature of the heat-  
 40 ed steam may vary for example from 5°—100° C. above the boiling point of water at the pressure obtaining, provided that the temperature in question does not reach the decomposition temperature of the cellulose  
 45 ester or ether contained in the material or

the scorching temperature of any other fibre which may be used in association.

As in the said prior United States applica-  
 50 tion a stretch may be imparted to the fila-  
 ments, yarns, fabrics or other products treat-  
 ed, either before or during the steaming  
 treatment. Again as in the said prior  
 United States application filaments or  
 55 threads of any type, for example flat or rib-  
 on-like filaments, semi-round and round  
 filaments and the so-called hollow, tubular or  
 voluminous filaments or threads may be  
 treated, and in addition any products made  
 60 therefrom with or without other fibres, for  
 example cotton, the cellulosic type of arti-  
 ficial silk or natural silk. The materials  
 treated according to the present invention  
 may be either completely delustered with re-  
 65 gard to their cellulose ester or ether content  
 or may be partially or locally delustered.  
 In the last case the process of the invention  
 renders the lustre of the materials substan-  
 tially uniform.

The following examples show the best  
 70 methods known to us for carrying the inven-  
 tion into effect but they are not to be consid-  
 ered as limiting it in any way:

## Example 1

75 Yarns of cellulose acetate artificial silk or fabrics made of or containing cellulose acetate  
 80 artificial silk alone or in admixture with cotton or natural silk and in the dyed or un-  
 dyed state, in which the cellulose acetate has  
 been delustered by treatment in a boiling soap  
 solution, are steamed for half an hour at a  
 85 pressure of 20 lbs. per square inch in excess  
 of atmospheric pressure and at a temperature  
 of 175 to 185° C. The lustre of the cellulose  
 acetate artificial silk is thereby restored.

## Example 2

90 A fabric composed of a real silk crêpe weft  
 and a cellulose acetate warp, which has been  
 much reduced in lustre by boiling in an aque-

ous soap solution, is formed into a series of loops and introduced into a steaming chamber fitted with a heated oil jacket and a steam supply with super heater. It is treated for 1 hour, the steam pressure being adjusted to 10 lbs. per square inch and the temperature to 180° C. The lustre of the fabric is restored.

*Example 3*

3 A garment made from fabric composed of cellulose acetate yarns, and which has been delustered in places owing to laundering in soap solution at too high a temperature, is placed in the dry state on a suitable form to preserve the shape and thus introduced into a steaming apparatus, as described in the above example. It is treated for 20 minutes with steam at 40 lbs. per square inch, the temperature being adjusted to 150° C. The lustre of the garment is restored.

What we claim and desire to secure by Letters Patent is:—

1. Process for increasing at least locally the lustre of the materials containing cellulose derivatives which have been delustered by the action of hot aqueous media, comprising subjecting the materials to the action of super-heated steam.

2. Process for increasing at least locally the 30 lustre of materials containing organic derivatives of cellulose which have been delustered by the action of hot aqueous media, comprising subjecting the materials to the action of super-heated steam.

3. Process for increasing at least locally the 35 lustre of materials containing cellulose acetate which have been delustered by the action of hot aqueous media, comprising subjecting the materials to the action of super-heated steam.

4. Process for increasing at least locally the 40 lustre of materials containing cellulose acetate which have been delustered by the action of hot aqueous media, comprising subjecting the materials to the action of super-heated steam which is at a temperature of 5 to 100° C. above the boiling point of water at the prevailing pressure of the steam.

5. Process for increasing at least locally the 45 lustre of materials containing organic derivatives of cellulose which have been delustered by the action of hot aqueous media, comprising subjecting the materials to the action of super-heated steam at pressures greater than atmospheric.

6. Process for increasing at least locally the 50 lustre of materials containing cellulose acetate which have been delustered by the action of hot aqueous media, comprising subjecting the materials to the action of super-heated steam at pressures greater than atmospheric.

7. Process for increasing at least locally the 55 lustre of materials containing cellulose acetate which have been delustered by the action of hot aqueous media, comprising subjecting

the materials to the action of super-heated steam at pressures greater than atmospheric which is at a temperature of 5 to 100° C. above the boiling point of water at the prevailing pressure of the steam.

In testimony whereof we have hereunto subscribed our names.

GEORGE HOLLAND ELLIS.  
HENRY CHARLES OLPIN.

70

75

80

85

90

95

100

105

110

115

120

125